# EUROPEAN PATENT SPECIFICATION

(11) **EP 4 287 227 B1**
(45) Date of publication and mention of the grant of the patent: **08.07.2026**
(21) Application number: 23174413.7
(22) Date of filing: 22.05.2023
(51) Int. Cl.: H01F 41/02, H01F 1/057

(54) **DIFFUSION SOURCE MATERIAL AND ITS USE FOR PREPARATION OF NDFEB MAGNETS**
DIFFUSIONSQUELLENMATERIAL UND DESSEN VERWENDUNG ZUR HERSTELLUNG VON NDFEB-MAGNETEN
MATÉRIAU SOURCE DE DIFFUSION ET SON UTILISATION POUR LA PRÉPARATION D'AIMANTS NDFEB

(30) Priority: 31.05.2022 CN 202210609436
(43) Date of publication of application: 06.12.2023
(73) Proprietor: Yantai Dongxing Magnetic Materials Inc., Yantai City 265500 (CN)
(72) Inventor: WANG, Chuanshen, Yantai City, 265500 (CN); PENG, Zhongjie, Yantai City, 265500 (CN); YANG, Kunkun, Yantai City, 265500 (CN); DONG, Zhanji, Yantai City, 265500 (CN); DING, Kaihong, Yantai City, 265500 (CN)
(74) Representative: Gulde & Partner

(56) References cited:
- CN-A- 112 802 677
- CN-B- 106 298 219
- JP-A- 2013 225 533

## Description

### BACKGROUND OF THE INVENTION

### 1. Field of the Invention

The invention relates to the technical field of NdFeB rare earth magnets, in particular to rare earth magnets with improved coercivity and its manufacturing method thereof. The invention further refers to a method of preparing a diffusion source material useful for preparing the NdFeB magnets.

### 2. Description of the Prior Art

NdFeB sintered permanent magnets are widely used in electronic equipment, medical equipment, electric vehicles, household products, robots, etc. In the past few decades of development, NdFeB permanent magnets and their manufacturing processes have been rapidly developed. In particular, a thermally induced diffusion process has been developed which could significantly reduce the consumption of heavy rare earths and has a large cost advantage.

When the heavy rare earth elements Dy or Tb are added to the base alloy during the production of sintered NdFeB permanent magnets, they are present in large quantities in the grain and the consumption of the heavy rare earth elements is correspondingly high. In addition, this leads to a reduction in the residual magnetism of the magnet. Therefore, an alternative method is the so-called grain boundary diffusion, in which a diffusion source is diffused into the magnet along the grain boundary to improve the coercivity of the magnet. This technology uses significantly less heavy rare earths while achieving the same coercivity of the magnets. The process has therefore become widely used in practice, if only for cost reasons. However, as the prices of the heavy rare earths Dy and Tb continue to rise due to very high demand, the cost of grain boundary diffusion technology using pure Dy and Tb is still very high. Therefore, continuous improvement of heavy rare earth alloy diffusion technology is particularly important for the mass production of NdFeB magnets.

US8801870B2 provides a method for making a NdFeB sintered magnet including the processes of coating a NdFeB sintered magnet with a powder containing R^{h} (where R^{h} represents Dy and/or Tb), then heating the NdFeB sintered magnet, and thereby diffusing R^{h} in the powder into the NdFeB sintered magnet through the grain boundaries. The powder contains 0.5 through 50 weight percent of Al in a metallic state; and the amount of oxygen contained in the NdFeB sintered magnet is equal to or less than 0.4 weight percent. However, the consumption of R^{H} is not reduced compared to the use of the pure elements to achieve the same coercivity effect.

In CN106298219B the diffusion source is an R^{L}ᵤR^{H}ᵥFe_{100-u-v-w-z}B_{w}M_{z} rare earth alloy. R^{L} represents at least one element of Pr and Nd, R^{H} represents at least one element in Dy, Tb, and Ho, M represents at least one element of Co, Nb, Cu, Al, Ga, Zr, and Ti, and u, v, w, z is in weight percentage 0≤u≤10, 35≤v≤70, 0.5≤w≤5, 0≤z≤5. The alloy is crushed to form alloy powders. The alloy powders are loaded into a rotary diffusion device with an R-T-B magnet for thermal diffusion in a temperature range of 750°C to 950°C for 4h to 72h, followed by an aging treatment. However, when the B content in the diffusion source is too high, its melting point will be relatively high and it is not easy to diffuse the alloy into the magnet. When the iron content is high in the magnet, too many ferromagnetic phases are formed, and the performance of the NdFeB magnet is reduced including the Hcj and Br of the magnet.

In CN113593800A the diffusion source is R^{H}ₓM¹_{y}B_{z}, where R^{H} is selected from one or two elements of Dy and Tb, M¹ is selected from one, two or three elements of Ti, Zr, and Al, B is boron, and x, y, z satisfies in weight percentages the following relationship: 75%≤x≤90%, 0.1%≤z≤0.5%, y=1-x-z. The method improves the Hcj of the sintered NdFeB magnet by diffusion and the coercivity is slightly improved. However, the longterm use of the diffusion source will inevitably cause certain oxidation and nitridation. Furthermore, when the diffusion source contains Ti or Zr, its melting point will be relatively high, resulting in a low diffusion rate. When consuming the same heavy rare earth content, the residual magnetism drops more, the coercivity of the magnet is not further improved.

JP 2013 225533 A and CN 112 802 677 A disclose methods of preparing sintered NdFeB magnets including a diffusion process.

### SUMMARY OF THE INVENTION

The invention is defined by the appended claims. The description that follows is subjected to this limitation. Any disclosure lying outside the scope of said claims is only intended for illustrative as well as comparative purposes.

### DETAILED DESCRIPTION OF THE INVENTION

Reference will now be made in detail to embodiments. The present disclosure, however, may be embodied in various different forms, and should not be construed as being limited to only the illustrated embodiments herein. Rather, these embodiments are provided as examples so that this disclosure will be thorough and complete, and will fully convey the aspects and features of the present disclosure to those skilled in the art.

There are provided a method of preparing a diffusion source material (Section A) and a method for preparing a NdFeB rare earth magnet (Section B).

### A. Production of the Diffusion Source Material

A novel method for preparing a diffusion source material, which is useful for preparing NdFeB magnets, is provided. The method comprises the following steps:
a) preparing an alloy sheet being of chemical formula R_{α}RH_{δ}M_{β}B_{γ}Fe_{100-α-β-γ-δ}, where R is at least one of Nd and Pr, and 10≤α≤50, preferably 15≤α≤45, RH is at least one of Dy and Tb and 25≤δ≤75, preferably 30≤δ≤70, M is at least one of Al, Cu, and Ga, and 5≤β≤30 preferably 10≤β≤25, B is boron and 0.3≤γ≤6, preferably 0.5≤γ≤5, and wherein the proportions are given in percentage by weight, the balance of the alloy being Fe and a proportion of Fe in the alloy is 2 to 12 percent by weight, preferably 3 to 11 percent by weight;
b) coating an alloy film on the alloy sheet, the alloy film being of chemical formula RₙMₘ, where R is at least one of Nd, Pr, Ce, and La, and 45≤n≤85, preferably 50≤n≤82, and M is at least one of Al, Cu, and Ga, and 15≤m≤55, preferably 18≤m≤50, wherein the proportions are given in percentage by weight and sum up to 100 percentage by weight and wherein a weight ratio of the weight of the alloy film to the weight of the diffusion source alloy sheet is in the range of 1:100 to 5:100, preferably 2:100 to 4:100;
c) performing a heat treatment of the coated alloy sheet; and
d) crushing the alloy sheet into a diffusion source material.

Alloy compositions of exemplary diffusion source materials, which may be used in step a) of the process, are summarized in **Table** 1. The alloy components forming the alloy sheet of Preparation Samples 1 to 18 were put into a vacuum melting furnace for melting. The melt was poured to form the alloy sheet, wherein the average thickness of the alloy sheet was about 0.25 mm. A content of C and O in the alloy sheet was ≤ 200ppm, and the N content was ≤ 50ppm.

In Preparation Samples 1 to 18, a surface of the alloy sheet was coated with a layer of non-heavy rare earth alloy film by using a spray-coating process. Other coating processes may be used, for example dip coating or screen-printing coating. The compositions of the alloy film in Preparation Samples 1 to 18 are also summarized in **Table 1.** The coated alloy sheets were put into a drying furnace for drying at a temperature of 80°C to 150°C. A weight ratio of the weight of the alloy film to the weight of the alloy sheet in Preparation Samples 1 to 18 was 3:100.

The heat treatment in step c) may be performed at a temperature of 600°C to 800°C for 2h to 10h. In Preparation Samples 1 to 18, the temperature was always at about 700°C for about 6h. The samples were actively cooled to about 40°C. The cooling method was rapid cooling using a circulating airflow, and the cooling gas atmosphere was argon. Other inert gases, such as helium, may be used.

The crushing of step d) may be performed by a hydrogen embrittlement process followed by a jet milling process. Specifically, the coated and thermally treated alloy sheet may be subjected to a hydrogen embrittlement process (i.e. hydrogen absorption and dehydrogenation), followed by jet milling for preparing powdered diffusion source material. The hydrogen embrittlement process, and the jet milling process are well-known technologies for the person skilled in the art and on the field of NdFeB magnet production. A hydrogen absorption temperature during the hydrogen embrittlement process may be 50°C to 200°C, and a dehydrogenation temperature during the hydrogen embrittlement process may be 450°C to 550°C. In Preparation Samples 1 to 18, the hydrogen absorption temperature was about 150°C, and the dehydrogenation temperature during the hydrogen embrittlement process was about 500°C.

The diffusion source material obtained by the process may have an average D50 particle size of 3µm to 60µm measured by laser diffraction after the crushing of step d). The average particle diameter D50 of the particles may be measured by laser diffraction (LD). The method may be performed according to ISO 13320-1. According to the IUPAC definition, the equivalent diameter of a non-spherical particle is equal to a diameter of a spherical particle that exhibits identical properties to that of the investigated non-spherical particle. In Preparation Samples 1 to 18, the average D50 particle size was about 8µm to 10µm.

### B. Production of the NdFeB Magnet

A method for preparing a NdFeB magnet comprises the following steps:
(S1) providing the diffusion source material as defined above;
(S2) providing a sintered NdFeB magnet; and
(S3) applying the diffusion source material on the surface of the sintered NdFeB magnet and performing a thermal diffusion process.

In step S2, a sintered NdFeB magnet is provided. A NdFeB magnet (also known as NIB or Neo magnet or NdFeB rare earth magnet) is the most widely used type of rareearth magnet. It is a permanent magnet made from an alloy of neodymium, iron, and boron to form the Nd2Fe14B tetragonal crystalline structure as a main phase. Besides, the microstructure of NdFeB magnets includes usually a Nd-rich phase. The alloy may include further elements in addition to or partly substituting neodymium and iron. The present invention may specifically refer to a sintered NdFeB magnet being formed of an NdFeB base alloy of chemical formula RₐM¹_{b}M²_{c}B_{d}Fe_{100-a-b-c-d}, where 27≤a≤33, 0.1≤b≤4, preferably 0.3≤b≤3, 0.5≤c≤3, preferably 0.5≤c≤2.15, 0.8≤d≤1.2, R refers to one or more of Dy, Tb, Y, Ho, Gd, Nd, Pr, Ce, and La, M¹ refers to one or more of Al, Cu, and Ga, M² refers to one or more of Ti, Zr, Co, Mg, Zn, Nb, Mo, and Sn, wherein the proportions are given in percentage by weight and the balance of the NdFeB base alloy being Fe. Specific alloy compositions of the NdFeB magnets are summarized in **Table 2** (Base Alloy Samples 1 to 18). The C, O content of Base Alloy Samples 1 to 18 was ≤ 200ppm, the N content was ≤ 50ppm.

The sintered NdFeB magnet may be produced according to a conventional process well-known in the art. Specifically, NdFeB alloy flakes of the desired alloy composition may be produced by a strip casting process (for example, using a vacuum induction furnace), then subjected to a hydrogen embrittlement process (i.e. hydrogen absorption and dehydrogenation), followed by jet milling for preparing NdFeB magnet powders. The strip casting process, the hydrogen embrittlement process, and the jet milling process are well-known technologies.

According to an embodiment, the hydrogen embrittlement process comprises a hydrogen absorption step and a dehydrogenation step. The hydrogen absorption step may be performed at a temperature in the range of 100°C to 300°C and the dehydrogenation step may be performed at a temperature in the range of 400°C to 600°C. During the hydrogen absorption step, the content of hydrogen content may be less than 1000ppm, and the content of oxygen may be less than 500ppm. Jet milling may be performed under an inert gas, in particular argon. The powder of Base Alloy Samples 1 to 18 had an average particle size D50 after jet milling of 2µm to 5µm. The average particle diameter D50 of the particles may be measured by laser diffraction (LD). The method may be performed according to ISO 13320-1. According to the IUPAC definition, the equivalent diameter of a non-spherical particle is equal to a diameter of a spherical particle that exhibits identical properties to that of the investigated non-spherical particle.

The NdFeB alloy powder is usually pressed to form a green compact (blank) while applying a magnetic field. The green compact is sintered. Further, thermally aging steps may follow to form a sintered NdFeB magnet. A temperature of the sintering process for preparing the NdFeB magnet base alloy may be 980°C to 1060°C at a sintering time of 6h to 15 h. Aging may be performed in two steps, for example, at a first aging temperature of 700°C to 850°C for 2h to 10h and a second aging temperature of 450°C to 600°C for 3h to 10h. In **Table 2,** characteristics of NdFeB magnets prior to the diffusion process are summarized.

In step S3, the diffusion source material is applied on the surface of the sintered NdFeB magnet and a thermal diffusion process is performed. Applying the diffusion source material may be achieved by any conventional process. For example, a slurry may be formed from powdered diffusion source material and a slurry forming component. The slurry may be coated on the sintered NdFeB magnet using a spray-coating process, a dip coating process or screen-printing process. In the diffusion process, the coated NdFeB magnet is heated to a diffusion temperature. Preferably, a diffusion temperature in step S3 is 850°C to 950°C and a diffusion time is 6h to 30h. Subsequently, aging may be performed. For example, a first aging temperature may be 700°C to 850°C for 2h to 10h and a second aging temperature may be 450°C to 600°C for 3h to 10h.

In **Table 3,** process conditions of the diffusion process and aging as well as characteristics of the NdFeB magnets after diffusion are summarized. In Example 1 the diffusion source material of Preparation Sample 1 was coated onto the Base Alloy Sample No. 1, in Example 2 the diffusion source material of Preparation Sample 2 was coated onto the Base Alloy Sample No. 2, etc.

The NdFeB magnets obtained by the process comprises a main phase, heavy rare earth shells, a grain boundary phase and a rare earth-rich phase. The grain boundary phase comprises a µ-phase and a δ-phase. The µ-phase is R_{36.5}Fe_{63.5-x}Mₓ with 2.5≤x≤5 and the δ-phase is R_{32.5}Fe_{67.5-y}M_{y} with 7≤y≤25, where R refers to at least two elements selected from Nd, Pr, Ce, and La, and M refers to at least two elements selected from Al, Cu, and Ga, wherein the proportions are given in atomic percentages. In each of Examples 1 to 18, a µ-phase and a δ-phase could be identified in the grain boundary phase.

In **Table 4,** diffusion source materials, process conditions and characteristics of Comparative Examples 1 to 18 are summarized. In Comparative Example 1 the mentioned diffusion source material of Table 4 was coated onto the Base Alloy Sample No. 1, in Comparative Example 2 the mentioned diffusion source material of Table 4 was coated onto the Base Alloy Sample No. 2, etc.

The residual magnetic reduction of the Examples was significantly lower than the Comparative Examples. Further, the coercivity of the Examples was higher than that of the Comparative Examples. The samples were analysed as follows:
Example 1 and Comparative Example 1: Example 1 shows Br = 1.330 T, Hcj = 2069.6 kA/m and contains a µ-phase and a δ-phase. Comparative Example 1 shows Br=1.315 T, Hcj=1990 kA/m and only contains the δ-phase.
Example 2 and Comparative Example 2: Example 2 shows Br=1.275 T, Hcj = 1830.8 kA/m and contains a µ-phase and a δ-phase. Comparative Example 2 shows Br= 1.260 T, Hcj=1791 kA/m and only contains the δ-phase.
Example 3 and Comparative Example 3: Example 3 shows Br=1.475 T, Hcj=1950.2 kA/m and contains a µ-phase and a δ-phase. Comparative Example 3 shows Br= 1.460 T, Hcj = 1830.8 kA/m and only contains the δ-phase.
Example 4 and Comparative Example 4: Example 4 shows Br= 1.465 T, Hcj = 1830.80 kA/m and contains a µ-phase and a δ-phase. Comparative Example 4 shows Br=1.450 T and Hcj=1751.2 kA/m.
Example 5 and Comparative Example 5: Example 5 shows Br=1.450 T, Hcj=1870.6 kA/m and contains a µ-phase and a δ-phase. Comparative Example 5 shows Br= 1.430 T and Hcj=1751.2 kA/m.
Example 6 and Comparative Example 6: Example 6 shows Br=1.435 T, Hcj=1990 kA/m and contains a µ-phase and a δ-phase. Comparative Example 6 shows Br= 1.420 T and Hcj=1950.2 kA/m.
Example 7 and Comparative Example 7: Example 7 shows Br=1.415 T, Hcj=2069.6 kA/m and contains a µ-phase and a δ-phase. Comparative Example 7 shows Br= 1.390 T and Hcj=1950.20 kA/m.
Example 8 and Comparative Example 8: Example 8 shows Br= 1.390 T, Hcj = 2228.80 kA/m and contains a µ-phase and a δ-phase. Comparative Example 8 shows Br=1.370 T and Hcj=2109.40 kA/m.
Example 9 and Comparative Example 9: Example 9 shows Br= 1.400 T, Hcj = 2109.40 kA/m and contains a µ-phase and a δ-phase. Comparative Example 9 shows Br=1.380 T and Hcj=1974.08 kA/m.
Example 10 and Comparative Example 10: Example 10 shows Br=1.345 T, Hcj= 2109.40 kA/m and contains a µ-phase and a δ-phase. Comparative Example 10 shows Br=1.330 T and Hcj=1950.20 kA/m and only contains the δ-phase.
Example 11 and Comparative Example 11: Example 11 shows Br=1.335 T, Hcj= 2149.2 kA/m and contains a µ-phase and a δ-phase. Comparative Example 11 shows Br=1.320 T and Hcj=1990 kA/m and only contains the δ-phase.
Example 12 and Comparative Example 12: Example 12 shows Br=1.385 T, Hcj= 2029.80 kA/m and contains a µ-phase and a δ-phase. Comparative Example 12 shows Br=1.365 T and Hcj=1870.60 kA/m.
Example 13 and Comparative Example 13: Example 13 shows Br=1.385 T, Hcj= 2467.60 kA/m and contains a µ-phase and a δ-phase. Comparative Example 13 shows Br=1.370 T and Hcj=2268.60 kA/m.
Example 14 and Comparative Example 14: Example 14 shows Br=1.375 T, Hcj= 2228.80 kA/m and contains a µ-phase and a δ-phase. Comparative Example 14 shows Br=1.360 T and Hcj=2109.40 kA/m.
Example 15 and Comparative Example 15: Example 15 shows Br=1.335 T, Hcj= 2149.2 kA/m and contains a µ-phase and a δ-phase. Comparative Example 15 shows Br=1.325 T and Hcj=1990.00 kA/m.
Example 16 and Comparative Example 16: Example 16 shows Br=1.340 T, Hcj= 2308.4 kA/m and contains a µ-phase and a δ-phase. Comparative Example 16 shows Br=1.325 T, Hcj=2149.20 kA/m and only contains the δ-phase.
Example 17 and Comparative Example 17: Example 17 shows Br=1.260 T, Hcj= 2308.4 kA/m and contains a µ-phase and a δ-phase. Comparative Example 17 shows Br=1.250 T, Hcj=2149.20 kA/m and only contains the δ-phase.
Example 18 and Comparative Example 18: Example 18 shows Br=1.360 T, Hcj= 2228.80 kA/m and contains a µ-phase and a δ-phase. Comparative Example 18 shows Br=1.345 T and Hcj=2109.40 kA/m.

The present invention ensures at least some of the following technical effects:
(1) The diffusion source material (i.e. alloy R_{α}RH_{δ}M_{β}B_{γ}Fe_{100-α-β-γ-δ} coated with RnMm alloy) reduces the proportion of Fe content, increases the proportion of M, and has a low content of high melting point B. The diffusion source material can effectively solve the problem of a low diffusion rate due to a small amount of B. This method can well transport heavy rare earths into the magnet, forming heavy rare earth shells, effectively increasing the coercivity of the magnet, and can well improve the diffusion speed.
(2) The diffusion source material contains elemental B, which can reduce the oxidation problem in the diffusion process, so as to increase the utilization efficiency of the elements in the diffusion process.
(3) The diffusion source material further contains B and Fe, which can form a main phase by diffusing into the magnet, thereby increasing the Br value. Increasing the Br value of the magnet can offset the large decrease in the Br value during the heavy earth diffusion process, and the residual magnetic decline is less than 0.015 T. The element of Fe can form a µ- and δ-phase with Al, Ga and Cu during the diffusion process, so as to improve the coercivity of the magnet. The decrease of Br is ≤ 0.15Kgs, the increase of coercivity Hcj is ≥ 8kOe, and the typical increase can reach 9kOe after diffusing the diffusion source material.
(4) The diffusion source material contains B and Fe, and the total weight ratio of B and Fe can reach up to 18%, which greatly reduces the price of the diffusion source, thereby reducing the total production costs.
(5) The diffusion source material can be prepared in large quantities, and the coating method can achieve nearly 100% utilization efficiency which can reduce production costs.
(6) The prepared NdFeB magnet base alloy is only sintered to form a sintered state, without the need for primary aging and secondary aging. It can reduce production costs very well. Compared with the prior art, the present invention realizes the cooperation between the diffusion source of heavy rare earth alloy and the corresponding component magnet, greatly improves the coercivity of the magnet, and reduces the problem of large Br decline.

**Table 1 - Composition of diffusion source materials**

| Preparation Sample No. | alloy sheet R_{α}RH_{δ}M_{β}B_{γ}Fe_{100-α-β-γ-δ} (wt.%) | alloy film RₙMₘ (wt.%) |
|---|---|---|
| 1 | Pr:30%, Tb:45%, Al:10%, B:4%, Fe: bal. | Pr:82% Ga:18% |
| 2 | Pr:30%, Tb:45%, Cu:15%, B:3%, Fe: bal. | Pr:70% Cu:20% Ga:10% |
| 3 | Nd:20%, Tb:45%, Al:12%, Cu:13%, B:3%, Fe: bal. | Pr:50% Cu:30% Ga:20% |
| 4 | Pr:30%, Dy:45%, Al:10%, Ga:5%, B:5%, Fe: bal. | Nd:60% Cu:40% |
| 5 | Pr:30%, Dy:45%, Ga:10%, Cu:5%, B:5%, Fe: bal. | Nd:70% Cu:20% Ga:10% |
| 6 | Nd:30%, Dy:45%, Cu:15%, B:2%, Fe: bal. | Pr:80% Al:20% |
| 7 | Pr:30%, Dy:50%, Ga:10%, B:1%, Fe: bal. | Nd:70% La:5% Cu:25% |
| 8 | Pr:20%, Tb:50%, Ga:10%, Cu:10%, B:3%, Fe: bal. | Pr:50% Ce:5% Cu:45% |
| 9 | Pr:15%, Dy:70%, Cu:10%, B:2%, Fe: bal. | Pr:75% La:6% Ga:19% |
| 10 | Pr:15%, Dy:70%, Al:10%, B:0.5%, Fe: bal. | Pr:60% Cu:40% |
| 11 | Pr:15%, Dy:70%, Al:5%, Cu:5%, B:1%, Fe: bal. | Pr:65% Ce:5% Cu:30% |
| 12 | Nd:25%, Dy:60%, Cu:10%, B:0.5%, Fe: bal. | Pr:75% Ga:25% |
| 13 | Nd:25%, Tb:60%, Cu:10%, B:2%, Fe: bal. | Pr:50% La:5% Cu:45% |
| 14 | Nd:45%, Tb:30%, Cu:10%, Al:10%, B:2%, Fe: bal. | Pr:75% La:6% Ga:19% |
| 15 | Nd:30%, Dy:50%, Cu:10%, Ga:3%, B:4%, Fe: bal. | Nd:70% Cu:30% |
| 16 | Pr:20%, Dy:40%, Tb:10%, Cu:10%, Al:5%, B:5%, Fe: bal. | Nd:65% Ce:5% Cu:30% |
| 17 | Pr:20%, Tb:40%, Dy:10%, Cu:10%, Al:5%, B:4%, Fe: bal. | Nd:50% Ga:10% Cu:40% |
| 18 | Pr:30%, Dy:40%, Tb:10%, Cu:10%, B:2%, Fe: bal. | Nd:50% Ga:25% Cu:25% |

**Table 2 - NdFeB base alloy compositions and its performance**

| | Composition of NdFeB base alloy (wt.%) | | | | | | | | | | | | | | | Performance | | |
|---|---|---|---|---|---|---|---|---|---|---|---|---|---|---|---|---|---|---|
| | R | | | | | | | M1 | | | M2 | | | | | | | |
| Base Alloy Sample No. | Pr | Nd | Ce | Ho | Gd | Dy | Tb | Cu | Al | Ga | Co | Ti | Zr | Fe | B | Br(T) | Hcj(kA/m) | Hk/Hcj |
| 1 | 6.19 | 24.75 | 2.00 | 0.00 | 0.00 | 0.00 | 0.00 | 0.29 | 0.40 | 0.10 | 1.00 | 0.05 | 0.00 | bal. | 0.92 | 1.340 | 1162.16 | 0.98 |
| 2 | 0.00 | 23.52 | 8.00 | 0.00 | 0.00 | 0.00 | 0.00 | 0.44 | 0.53 | 0.21 | 1.00 | 0.20 | 0.05 | bal. | 0.94 | 1.280 | 915.40 | 0.98 |
| 3 | 0.00 | 29.50 | 0.00 | 0.00 | 0.00 | 0.00 | 0.00 | 0.15 | 0.05 | 0.10 | 0.90 | 0.00 | 0.10 | bal. | 0.92 | 1.485 | 955.20 | 0.98 |
| 4 | 7.70 | 21.92 | 0.00 | 0.00 | 0.00 | 0.00 | 0.00 | 0.16 | 0.06 | 0.09 | 1.50 | 0.00 | 0.08 | bal. | 0.91 | 1.473 | 1106.44 | 0.98 |
| 5 | 0.00 | 29.20 | 0.00 | 0.00 | 0.00 | 0.00 | 0.30 | 0.15 | 0.05 | 0.20 | 1.00 | 0.10 | 0.00 | bal. | 0.94 | 1.460 | 1194.00 | 0.98 |
| 6 | 7.51 | 22.27 | 0.00 | 0.00 | 0.00 | 0.00 | 0.00 | 0.21 | 0.11 | 0.20 | 1.94 | 0.01 | 0.00 | bal. | 0.90 | 1.440 | 1305.44 | 0.98 |
| 7 | 6.46 | 23.70 | 0.00 | 0.00 | 0.00 | 0.00 | 0.00 | 0.15 | 0.20 | 0.20 | 1.31 | 0.14 | 0.00 | bal. | 0.95 | 1.427 | 1273.60 | 0.98 |
| 8 | 7.50 | 23.20 | 0.00 | 0.00 | 0.00 | 0.00 | 0.00 | 0.16 | 0.23 | 0.21 | 0.91 | 0.15 | 0.00 | bal. | 0.95 | 1.398 | 1313.40 | 0.99 |
| 9 | 6.26 | 25.04 | 0.00 | 0.00 | 0.00 | 0.00 | 0.00 | 0.15 | 0.20 | 0.20 | 1.50 | 0.10 | 0.00 | bal. | 0.94 | 1.410 | 1278.38 | 0.98 |
| 10 | 7.70 | 23.70 | 0.00 | 0.00 | 0.00 | 0.00 | 0.00 | 0.15 | 0.60 | 0.22 | 1.00 | 0.10 | 0.05 | bal. | 0.90 | 1.360 | 1393.00 | 0.99 |
| 11 | 6.24 | 24.96 | 0.00 | 0.00 | 0.00 | 0.00 | 0.00 | 0.30 | 0.80 | 0.20 | 1.00 | 0.10 | 0.00 | bal. | 0.98 | 1.346 | 1416.88 | 0.99 |
| 12 | 0.13 | 31.44 | 0.00 | 0.00 | 0.00 | 0.00 | 0.00 | 0.20 | 0.27 | 0.24 | 1.00 | 0.15 | 0.00 | bal. | 0.94 | 1.390 | 1273.60 | 0.98 |
| 13 | 5.98 | 23.92 | 0.00 | 0.00 | 0.00 | 0.00 | 1.10 | 0.01 | 0.20 | 0.30 | 1.00 | 0.05 | 0.04 | bal. | 0.91 | 1.395 | 1552.20 | 0.98 |
| 14 | 0.24 | 31.23 | 0.00 | 0.00 | 0.00 | 0.00 | 0.00 | 0.18 | 0.43 | 0.23 | 1.97 | 0.18 | 0.00 | bal. | 0.97 | 1.375 | 1353.20 | 0.98 |
| 15 | 5.90 | 24.18 | 0.00 | 1.00 | 0.00 | 0.00 | 0.00 | 0.18 | 0.30 | 0.18 | 0.50 | 0.18 | 0.00 | bal. | 0.93 | 1.340 | 1476.58 | 0.99 |
| 16 | 5.60 | 23.21 | 0.00 | 0.88 | 0.00 | 0.86 | 0.00 | 0.20 | 0.37 | 0.25 | 1.00 | 0.14 | 0.00 | bal. | 0.95 | 1.350 | 1512.40 | 0.98 |
| 17 | 6.06 | 23.17 | 0.00 | 0.00 | 2.60 | 0.00 | 0.00 | 0.16 | 0.95 | 0.31 | 1.53 | 0.10 | 0.00 | bal. | 0.94 | 1.266 | 1521.95 | 0.99 |
| 18 | 5.43 | 23.00 | 0.00 | 1.35 | 0.00 | 0.55 | 0.00 | 0.20 | 0.30 | 0.25 | 1.00 | 0.15 | 0.00 | bal. | 0.94 | 1.370 | 1432.80 | 0.98 |

**Table 3 - Process conditions and characteristics of the NdFeB magnets after diffusion of Examples 1 to 18**

| Example No. | Size | Diffusion temp. | Holding time | First aging temp. | Holding time | Second aging temp. | Holding time | Performance after diffusion | | | whether it contains µ-phase | whether it contains δ-phase |
|---|---|---|---|---|---|---|---|---|---|---|---|---|
| | mm | °C | h | °C | h | °C | h | Br T | Hcj kA/m | Hk/Hcj | | |
| 1 | 10*10*3 | 850 | 30 | 700 | 2 | 510 | 10 | 1.33 | 2069.6 | 0.97 | Yes | Yes |
| 2 | 10*10*4 | 900 | 15 | 700 | 3 | 480 | 7 | 1.275 | 1830.8 | 0.96 | Yes | Yes |
| 3 | 10*10*3 | 850 | 30 | 700 | 5 | 500 | 5 | 1.475 | 1950.2 | 0.96 | Yes | Yes |
| 4 | 10*10*3 | 900 | 10 | 700 | 8 | 530 | 8 | 1.465 | 1830.8 | 0.97 | Yes | Yes |
| 5 | 10*10*4 | 900 | 20 | 750 | 10 | 540 | 6 | 1.45 | 1870.6 | 0.97 | Yes | Yes |
| 6 | 10*10*4 | 910 | 20 | 750 | 2 | 600 | 5 | 1.435 | 1990 | 0.96 | Yes | Yes |
| 7 | 10*10*4 | 920 | 20 | 750 | 3 | 500 | 3 | 1.415 | 2069.6 | 0.97 | Yes | Yes |
| 8 | 10*10*4 | 910 | 15 | 750 | 5 | 460 | 6 | 1.39 | 2228.8 | 0.97 | Yes | Yes |
| 9 | 10*10*5 | 930 | 16 | 800 | 8 | 450 | 8 | 1.4 | 2109.4 | 0.96 | Yes | Yes |
| 10 | 10*10*5 | 940 | 10 | 800 | 10 | 520 | 6 | 1.345 | 2109.4 | 0.97 | Yes | Yes |
| 11 | 10*10*5 | 930 | 20 | 800 | 2 | 600 | 5 | 1.335 | 2149.2 | 0.97 | Yes | Yes |
| 12 | 10*10*6 | 950 | 20 | 800 | 3 | 500 | 8 | 1.385 | 2029.8 | 0.97 | Yes | Yes |
| 13 | 10*10*4 | 910 | 15 | 800 | 5 | 450 | 8 | 1.385 | 2467.6 | 0.97 | Yes | Yes |
| 14 | 10*10*3 | 850 | 10 | 850 | 8 | 500 | 6 | 1.375 | 2228.8 | 0.96 | Yes | Yes |
| 15 | 10*10*8 | 950 | 30 | 850 | 10 | 520 | 10 | 1.335 | 2149.2 | 0.96 | Yes | Yes |
| 16 | 10*10*3 | 910 | 10 | 850 | 3 | 500 | 5 | 1.34 | 2308.4 | 0.97 | Yes | Yes |
| 17 | 10*10*3 | 930 | 6 | 850 | 5 | 600 | 3 | 1.26 | 2308.4 | 0.96 | Yes | Yes |
| 18 | 10*10*5 | 940 | 8 | 850 | 8 | 580 | 8 | 1.36 | 2228.8 | 0.97 | Yes | Yes |

**Table 4 - Diffusion sources, process conditions and characteristics of the NdFeB magnets after diffusion of Comparative Example 1 to 18**

| Comparative Example No. | Diffusion source | Size | Diffusion Temp. | Holding time | Aging Temp. | Holdin g time | Performance after Diffusion | | | Whether it contains µ phase | Whether it contains δ phase |
|---|---|---|---|---|---|---|---|---|---|---|---|
| | | mm | °C | h | °C | h | Br | Hcj | Hk/Hcj | | |
| 1 | Pr:45%, Tb:45%, Al:10% | 10*10*3 | 850 | 30 | 510 | 10 | 1.315 | 1990.00 | 0.97 | NO | Yes |
| 2 | Pr:40%, Tb:45%, Cu:15% | 10*10*4 | 900 | 15 | 480 | 7 | 1.260 | 1791.00 | 0.96 | NO | Yes |
| 3 | Nd:30%, Tb:45%, Al:12%, Cu:13%, | 10*10*3 | 850 | 30 | 500 | 5 | 1.460 | 1830.80 | 0.96 | NO | NO |
| 4 | Pr:40%, Dy:45%, Al:10%, Ga:5% | 10*10*3 | 900 | 10 | 530 | 8 | 1.450 | 1751.20 | 0.97 | NO | NO |
| 5 | Pr:40%, Dy:45%, Ga:10%, Cu:5% | 10*10*4 | 900 | 20 | 540 | 6 | 1.430 | 1751.20 | 0.97 | NO | NO |
| 6 | Nd:40%, Dy:45%, Cu:15% | 10*10*4 | 910 | 20 | 600 | 5 | 1.420 | 1950.20 | 0.96 | NO | NO |
| 7 | Pr:40%, Dy:50%, Ga:10% | 10*10*4 | 920 | 20 | 500 | 3 | 1.390 | 1950.20 | 0.97 | NO | NO |
| 8 | Pr:30%, Tb:50%, Ga:10%, Cu:10% | 10*10*4 | 910 | 15 | 460 | 6 | 1.370 | 2109.40 | 0.96 | NO | NO |
| 9 | Pr:20%, Dy:70%, Cu:10% | 10*10*5 | 930 | 16 | 450 | 8 | 1.380 | 1974.08 | 0.96 | NO | NO |
| 10 | Pr:20%, Dy:70%, Al: 10% | 10*10*5 | 940 | 10 | 520 | 6 | 1.330 | 1950.20 | 0.97 | NO | Yes |
| 11 | Pr:20%, Dy:70%, Al:5%, Cu:5% | 10*10*5 | 930 | 20 | 600 | 5 | 1.320 | 1990.00 | 0.97 | NO | Yes |
| 12 | Nd:30%, Dy:60%, Cu:10% | 10*10*6 | 950 | 20 | 500 | 8 | 1.365 | 1870.60 | 0.97 | NO | NO |
| 13 | Nd:30%, Tb:60%, Cu:10% | 10*10*4 | 910 | 15 | 450 | 8 | 1.370 | 2268.60 | 0.96 | NO | Yes |
| 14 | Nd:50%, Tb:30%, Cu:10%, Al:10% | 10*10*3 | 850 | 10 | 500 | 6 | 1.360 | 2109.40 | 0.97 | NO | NO |
| 15 | Nd:37%, Dy:50%, Cu:10%, Ga:3% | 10*10*8 | 950 | 30 | 520 | 10 | 1.325 | 1990.00 | 0.97 | NO | NO |
| 16 | Pr:35%, Dy:40%, Tb:10%, Cu:10%, Al:5% | 10*10*3 | 910 | 10 | 500 | 5 | 1.325 | 2149.20 | 0.97 | NO | Yes |
| 17 | Pr:35%, Tb:40%, Dy:10%, Cu:10%, Al:5% | 10*10*3 | 930 | 6 | 600 | 3 | 1.250 | 2149.20 | 0.96 | NO | Yes |
| 18 | Pr:40%, Dy:40%, Tb:10%, Cu:10% | 10*10*5 | 940 | 8 | 580 | 8 | 1.345 | 2109.40 | 0.97 | NO | NO |

## Claims

1. A method of preparing a diffusion source material useful for preparing NdFeB magnets, the method comprising the following steps:
a) preparing an alloy sheet being of chemical formula R_{α}RH_{δ}M_{β}B_{γ}Fe_{100-α-β-γ-δ}, where
R is at least one of Nd and Pr, and 10≤α≤50,
RH is at least one of Dy and Tb and 25≤δ≤75,
M is at least one of Al, Cu, and Ga, and 5≤β≤30,
B is boron and 0.3≤γ≤6, and
wherein the proportions are given in percentage by weight, the balance of the alloy being Fe and a proportion of Fe in the alloy is 2 to 12 percent by weight;
b) coating an alloy film on the alloy sheet, the alloy film being of chemical formula RₙMₘ, where
R is at least one of Nd, Pr, Ce, and La, and 45≤n≤85, and
M is at least one of Al, Cu, and Ga, and 15≤m≤55,
wherein the proportions are given in percentage by weight and sum up to 100 percentage by weight and wherein a weight ratio of the weight of the alloy film to the weight of the diffusion source alloy sheet is in the range of 1:100 to 5:100;
c) performing a heat treatment of the coated alloy sheet; and
d) crushing the alloy sheet into a diffusion source material.

2. The method of claim 1, wherein the heat treatment in step c) is performed at a temperature of 600°C to 800°C for 2h to 10h.

3. The method of claim 1 or 2, wherein the crushing of step d) is performed by a hydrogen embrittlement process followed by a jet milling process.

4. The method of claim 3, wherein a hydrogen absorption temperature during the hydrogen embrittlement process is 50°C to 200°C, and a dehydrogenation temperature during the hydrogen embrittlement process is 450°C to 550°C.

5. The method of any one of the preceding claims, wherein the diffusion source material has an average D50 particle size of 3µm to 60µm measured by laser diffraction after the crushing of step d).

6. A method of preparing a NdFeB magnet, the method comprising the following steps:
(S1) providing a diffusion source material obtained by the method of claim 1;
(S2) providing a sintered NdFeB magnet; and
(S3) applying the diffusion source material on the surface of the sintered NdFeB magnet and performing a thermal diffusion process.

7. The method of claim 6, wherein the sintered NdFeB magnet is formed of an NdFeB base alloy of chemical formula RₐM¹_{b}M²_{c}B_{d}Fe_{100-a-b-c-d}, where 27≤a≤33, 0.1≤b≤4, 0.5≤c≤3, 0.8≤d≤1.2, R refers to one or more of Dy, Tb, Y, Ho, Gd, Nd, Pr, Ce, and La, M¹ refers to one or more of Al, Cu, and Ga, M² refers to one or more of Ti, Zr, Co, Mg, Zn, Nb, Mo, and Sn, wherein the proportions are given in percentage by weight and the balance of the NdFeB base alloy being Fe.

8. The method of claim 6 or 7, wherein a diffusion temperature in step (S3) is 850°C to 950°C, a diffusion time is 6h to 30h, a first-stage aging temperature is 700°C to 850°C, a first-level aging time is 2h to 10h, a second-stage aging temperature is 450°C to 600°C, and a second-stage aging time is 3h to 10h.

## Patentansprüche

1. Verfahren zum Herstellen eines Diffusionsquellenmaterials, das nützlich für das Herstellen von NdFeB-Magneten ist, wobei das Verfahren die folgenden Schritte umfasst:
a) Herstellen eines Legierungsblechs mit der chemischen Formel R_{α}RH_{δ}M_{β}B_{γ}Fe_{100-α-β-γ-δ}, wobei
R mindestens eines von Nd und Pr ist und 10≤α≤50,
RH mindestens eines von Dy und Tb ist und 25≤δ≤75,
M mindestens eines von Al, Cu und Ga ist und 5≤β≤30,
B Bor ist und 0,3≤γ≤6, und
wobei die Anteile in Gewichtsprozent angegeben sind, der Rest der Legierung Fe ist und der Anteil von Fe in der Legierung 2 bis 12 Gewichtsprozent beträgt;
b) Beschichten des Legierungsblechs mit einem Legierungsfilm, wobei der Legierungsfilm die chemische Formel RₙMₘ aufweist, wobei R mindestens eines von Nd, Pr, Ce und La ist und 45≤n≤85, und
M mindestens eines von Al, Cu und Ga ist und 15≤ m≤55,
wobei die Anteile in Gewichtsprozent angegeben sind und sich auf 100 Gewichtsprozent summieren und wobei ein Gewichtsverhältnis des Gewichts des Legierungsfilms zum Gewicht des Diffusionsquellenlegierungsblechs im Bereich von 1:100 bis 5:100 liegt;
c) Durchführen einer Wärmebehandlung des beschichteten Legierungsblechs; und
d) Zerstoßen des Legierungsblechs in ein Diffusionsquellenmaterial.

2. Verfahren nach Anspruch 1, wobei die Wärmebehandlung in Schritt c) bei einer Temperatur von 600 °C bis 800 °C für 2 h bis 10 h durchgeführt wird.

3. Verfahren nach Anspruch 1 oder 2, wobei das Zerstoßen in Schritt d) durch einen Wasserstoffversprödungsprozess, dem ein Strahlmahlprozess folgt, durchgeführt wird.

4. Verfahren nach Anspruch 3, wobei eine Wasserstoffabsorptionstemperatur während des Wasserstoffversprödungsprozesses 50 °C bis 200 °C beträgt und eine Dehydrierungstemperatur während des Wasserstoffversprödungsprozesses 450 °C bis 550 °C beträgt.

5. Verfahren nach einem der vorhergehenden Ansprüche, wobei das Diffusionsquellenmaterial eine durchschnittliche D50-Partikelgröße von 3 µm bis 60 µm aufweist, gemessen durch Laserbeugung nach dem Zerstoßen in Schritt d).

6. Verfahren zum Herstellen eines NdFeB-Magneten, wobei das Verfahren die folgenden Schritte umfasst:
(S1) Bereitstellen eines Diffusionsquellenmaterials, das durch das Verfahren nach Anspruch 1 erhalten wird;
(S2) Bereitstellen eines gesinterten NdFeB-Magneten; und
(S3) Aufbringen des Diffusionsquellenmaterials auf die Oberfläche des gesinterten NdFeB-Magneten und Durchführen eines Wärmediffusionsprozesses.

7. Verfahren nach Anspruch 6, wobei der gesinterte NdFeB-Magnet aus einer NdFeB-Basislegierung der chemischen Formel RₐM¹_{b}M²_{c}B_{d}Fe_{100-a-b-c-d} ausgebildet ist, wobei 27≤a≤33, 0,1≤b≤4, 0,5≤c≤3, 0,8≤d≤1,2, sich R auf eines oder mehrere von Dy, Tb, Y, Ho, Gd, Nd, Pr, Ce und La bezieht, sich M¹ auf eines oder mehrere von Al, Cu und Ga bezieht, sich M² auf eines oder mehrere von Ti, Zr, Co, Mg, Zn, Nb, Mo und Sn bezieht, wobei die Anteile in Gewichtsprozent angegeben sind und der Rest der NdFeB-Basislegierung Fe ist.

8. Verfahren nach Anspruch 6 oder 7, wobei eine Diffusionstemperatur in Schritt (S3) 850 °C bis 950 °C beträgt, eine Diffusionszeit 6 h bis 30 h beträgt, eine Alterungstemperatur einer ersten Stufe 700 °C bis 850 °C beträgt, eine Alterungszeit eines ersten Niveaus 2 h bis 10 h beträgt, eine Alterungstemperatur einer zweiten Stufe 450 °C bis 600 °C beträgt und eine Alterungszeit der zweiten Stufe 3 h bis 10 h beträgt.

## Revendications

1. Procédé de préparation d'un matériau source de diffusion utile pour la préparation d'aimants NdFeB, le procédé comprenant les étapes suivantes :
a) préparer une feuille d'alliage étant de formule chimique R_{α}RH_{δ}M_{β}B_{γ}Fe_{100-α-β-γ-δ}, où
R est au moins l'un de Nd et Pr, et 10≤α≤50,
RH est au moins l'un de Dy et Tb et 25≤δ≤75,
M est au moins l'un de Al, Cu et Ga, et 5≤β≤30,
B est le bore et 0,3≤γ≤6, et
dans lequel les proportions sont données en pourcentage en poids, le reste de l'alliage étant Fe et une proportion de Fe dans l'alliage étant de 2 à 12 pour cent en poids ;
b) revêtir un film d'alliage sur la feuille d'alliage, le film d'alliage étant de formule chimique RₙMₘ, où
R est au moins l'un de Nd, Pr, Ce et La, et 45≤n≤85, et
M est au moins l'un de Al, Cu et Ga, et 15≤m≤55,
dans lequel les proportions sont exprimées en pourcentage en poids et s'élèvent à 100 pourcentage en poids et dans lequel un rapport de poids du poids du film d'alliage au poids de la feuille d'alliage source de diffusion est compris entre 1:100 et 5:100 ;
c) effectuer un traitement thermique de la feuille d'alliage revêtue ; et
d) broyer la feuille d'alliage en un matériau source de diffusion.

2. Procédé de la revendication 1, dans lequel le traitement thermique de l'étape c) est effectué à une température de 600°C à 800°C pendant 2h à 10h.

3. Procédé de la revendication 1 ou 2, dans lequel le broyage de l'étape d) est effectué par un processus de fragilisation par l'hydrogène suivi d'un processus de broyage par jet.

4. Procédé de la revendication 3, dans lequel une température d'absorption d'hydrogène pendant le processus de fragilisation par l'hydrogène est comprise entre 50°C et 200°C, et une température de déshydrogénation pendant le processus de fragilisation par l'hydrogène est comprise entre 450°C et 550°C.

5. Procédé de l'une quelconque des revendications précédentes, dans lequel le matériau source de diffusion présente une taille de particules D50 moyenne de 3µm à 60µm mesurée par diffraction laser après le broyage de l'étape d).

6. Procédé de préparation d'un aimant NdFeB, le procédé comprenant les étapes suivantes :
(S1) fournir un matériau source de diffusion obtenu par le procédé de la revendication 1 ;
(S2) fournir un aimant NdFeB fritté ; et
(S3) appliquer le matériau source de diffusion sur la surface de l'aimant NdFeB fritté et effectuer un processus de diffusion thermique.

7. Procédé de la revendication 6, dans lequel l'aimant NdFeB fritté est formé d'un alliage de base NdFeB de formule chimique RₐM¹_{b}M²_{c}B_{d}Fe_{100-a-b-c-d}, où 27≤a≤33, 0,1≤b≤4, 0,5≤c≤3, 0,8≤d≤1,2, R se réfère à un ou plusieurs parmi Dy, Tb, Y, Ho, Gd, Nd, Pr, Ce et La, M¹ se réfère à un ou plusieurs parmi Al, Cu et Ga, M² se refère à un ou plusieurs parmi Ti, Zr, Co, Mg, Zn, Nb, Mo et Sn, dans lequel les proportions sont données en pourcentage en poids et le reste de l'alliage de base NdFeB étant Fe.

8. Procédé de la revendication 6 ou 7, dans lequel une température de diffusion à l'étape (S3) est de 850°C à 950°C, un temps de diffusion est de 6h à 30h, une température de vieillissement de première étape est de 700°C à 850°C, un temps de vieillissement de premier niveau est de 2h à 10h, une température de vieillissement de deuxième étape est de 450°C à 600°C, et un temps de vieillissement de deuxième étape est de 3h à 10h.
